

## UNITED STATES PATENT OFFICE.

BY RAMJI D. SAKLATWALLA, OF CRAFTON, PENNSYLVANIA.

## MANUFACTURE OF ALLOY STEEL AND IRON.

No Drawing.

Application filed July 16, 1924. Serial No. 726,335.

The present invention relates to the manufacture of alloy steel or iron, and more particularly to the reduction of the alloying elements directly from their ores, and 5 the production of the respective alloy steels and irons, without the introduction of excess carbon in the finished steel or iron.

In the manufacture of alloy steels and irons, under the practice heretofore prevalent, the alloying elements, in the already reduced metallic state, mostly in the form of a ferro-alloy, are added to a molten bath of steel or iron. For example, to obtain the 10 respective steels thereof, ferro-manganese, ferro-chromium, ferro-titanium, ferro-tungsten, ferro-vanadium, ferro-uranium, ferro-molybdenum, ferro-nickel, or metallic nickel and ferro-cobalt or cobalt metal, are added 15 to steel, in the molten state in the furnace, or after it is tapped in the ladle. As the 20 regular commercial grades of such ferro-alloys contain an appreciable amount of carbon, this practice introduces an undue amount of carbon in the steel. If the special 25 grades of low-carbon ferro-alloys are used, the cost of such alloys is comparatively so high as to prohibitively increase the cost 30 of steel produced. These defects are especially apparent in the case of steels where the content of the alloying element has to 35 be high and the carbon content low, as in the case of the so-called "stainless" or "rustless" steels or irons, which have a chromium content of over 8% combined with a low carbon content.

It is not commercially practicable to use the regular high carbon ferro-alloys, and then decarbonize the steels after their addition, as the process of oxidizing the carbon 40 is accompanied by an oxidation, and consequent waste, of the valuable alloying elements.

Another deficiency of the usual existing methods of manufacturing alloy steels, by 45 the addition of metallic ferro-alloys to molten steel, is the phenomenon of segregation. The alloy being added in the solid state in the form of lumps scattered over the surface of the molten steel, causes points 50 of concentration of the alloying elements at the location of each of the lumps. As the steel is tapped immediately after melting of the lumps in order to avoid an undue oxidation of the alloying elements, these 55 points of higher concentration have no op-

portunity to equalize themselves over the entire mass of metal by diffusion. Moreover, the ferro-alloys have various constituents of different melting points and degrees of solubility, as, for example, the carbides in the ordinary grades of alloy. Such carbides have a higher melting point than the remainder of the alloy. Such a carbide-containing ferro-alloy, when added to molten steel, will have the result that when the 60 rest of the alloy will be completely assimilated, the carbide content will still be in the solid state, floating in the molten steel, without giving up its alloying element content to the bath. Such solid particles with a 65 high alloying element content will persist in the steel on solidification and present segregation.

The above mentioned difficulties are overcome in the so-called "direct reduction" 70 process by adding the alloying element to the bath of molten steel or iron in the form of oxide or ore and reducing it with a reducing agent incorporated in the steel. The reducing agent and the alloying material 75 are added to a bath of steel consisting of a molten metal layer with a supernatant molten layer of slag, in such a manner that the alloying material is incorporated in the slag layer and the reducing agent is incorporated in the metal layer, and each thoroughly disseminated in their respective layers. With the alloying material, either 80 mixed together or separately, are added fluxing materials which combine with the 85 oxidation products of the reducing agent, thus effecting its removal from the finished steel or iron and which also combine with the metalloids present in the molten steel, thus effecting a refining of the steel simultaneously with the alloying procedure. To 90 effectively remove the last traces of the reducing agent, and especially of carbon, the temperature at the end of the alloying and refining process is raised, which greatly 95 accelerates the chemical reactions taking place.

If the total quantity of alloying material, such, for example, as chrome ore and fluxes 100 is added at one time, owing to the refractory nature of the ore, it is a difficult matter to melt it down into the slag layer and obtain a thorough dissemination. To overcome this 105 difficulty only a certain amount of the ore and fluxes is charged at one time and the 110

necessary reducing agent, which may be of an exothermic nature or be carbonaceous, or be a metallic carbide, or a mixture of them, is added in quantity proportional to reduce 5 the chrome oxide present in the slag layer. The reaction is then allowed to proceed between the slag layer and the metal layer, whereby the products of oxidation of the reducing agent, for instance, silica in case 10 silicon was used as the reducing agent, transfer into the slag layer, helping to liquefy and flux the contents of the slag layer. As soon as the slag layer has assumed a visible fluidity owing to the combination of the 15 silica with the fluxes and gangue material of the ore, more alloying material is charged into the slag layer until the same has again assumed a viscous appearance. Then the corresponding amount of silicon is charged 20 into the metal layer and the reaction allowed to take place until the slag layer has again assumed perfect fluidity. The operation of charging alloying material and reducing agent successively is then continued until 25 the necessary amount of alloying element has been incorporated in the molten steel or iron. Thus, by charging the alloying material and reducing agent in successive portions, a visual means is obtained, by watching 30 the fluidity of the slag layer, to following the alloying procedure and also to curtail the time of the alloying procedure as the alloying material will be liquefied by the help of chemical combination with the products of oxidation of the reducing agent and 35 not by heat alone. By this procedure, therefore, heat energy will be saved.

Also by this procedure, after each successive step of alloying, the dead slag can be 40 removed to a very great extent so that the useful furnace contents volume will not be occupied by waste slag. Thus a larger amount of steel can be melted and alloyed in this manner than if all the alloying material 45 were charged in one portion. This fact is of special importance, where the steel or iron has to be alloyed to contain several percent of alloying metal, as in the case of the high-chromium "stainless" or "rustless" steels or 50 irons.

The slag to which the successive charges of ore are added is very fluid, due to the silica introduced into it by the oxidation of the silicon reducing agent. The strong fluxing 55 action of the silica permits highly refractory ores to be charged into and assimilated by the slag. The highly fluid slag is chemically active and the simultaneous refining of the steel by the removal of the 60 objectionable metalloids, sulphur and phosphorus, is facilitated as well as the reduction of the alloying ore. Moreover, the fluidity of the slag causes a better circulation of the slag over the entire bath, thus giving 65 less chance of segregations.

The reduced alloying metal is in contact with the molten steel or iron at the moment of its reduction, or in its "nascent" state, consequently the best conditions are obtained for the alloying and uniform dissemination of the alloying metal throughout the steel. The alloying metal is obtained from a cheap source. The introduction of carbon and segregation are avoided in the finished 70 steel. 75

The process may be carried out in the following manner:

The steel or iron, to which the alloying element is to be added, is melted down with the necessary fluxes, decarbonizing agents, 80 etc. in an ordinary steel-making furnace, such as an open-hearth furnace, electric furnace, or other suitable furnace, so that a molten layer of metal with a supernatant layer of slag is obtained. To this furnace 85 bath is then added a portion of the raw alloying material, for instance, chrome ore, together with fluxes. Sufficient temperature is maintained in the furnace to enable the added materials to melt into the slag layer, forming a viscous liquid. Without waiting to perfectly liquefy this mass the calculated amount or a quantity slightly less than the theoretical amount of reducing agent, such, 90 for example, as silicon in the form of ferro-silicon, is then charged into the furnace. The ferro-silicon sinks through the slag layer and becomes incorporated in the metal layer. Reaction then sets in, between the metal layer 95 and the slag layer, whereby the slag layer 100 gradually assumes increased fluidity as the silica formed enters into this layer. When the slag layer assumes total fluidity, the next successive portion of chrome ore and flux is charged followed by the equivalent 105 charge of ferro-silicon. This operation is repeated until a sample taken of the molten steel shows the desired chromium content. Then the temperature of the furnace is increased momentarily, if an electric furnace, 110 by increasing the power input, to remove the last traces of silicon and carbon and the metal is tapped.

The successive charges of the reducing agent and alloying ore may be either charges 115 consisting of the reducing agent and ore mixed together, or the reducing agent and ore may be added in charges which are separate as well as successive. It is preferred to add the reducing agent and the ore in separate as well as successive charges, as the reaction may be kept under a better regulated control thereby. By "successive charging" I mean adding the materials in charges separated by sufficient time intervals to allow the reducing reaction to proceed to a substantial extent, and preferably toward completion, 120 before further charges are added.

As fluxes with the chrome ore may be used, lime, limestone, fluorspar, borax, soda- 125

ash or other well known fluxes depending on the composition of the gangue material of the ore.

The most generally adapted metallic reducing agent is ferro-silicon. However, silicon metal or any other silicon alloy, such as a silicon alloy containing one of the alloying metals, may also be advantageously used. For instance, in the case of the manufacture of socalled "stainless" steel a silicon-chromium alloy may be incorporated in the molten steel and its silicon content utilized to reduce a further quantity of chromium from chrome ore added to the bath. This procedure is especially advantageous in the case of a steel containing a high percentage of the alloying element.

In the case of alloy steels containing a plurality of alloying elements, this procedure may be carried out in the same manner, the raw materials in the right proportions, containing the plural alloying elements, being charged together in each successive batch, or separately in the successive batches, on top of the molten bath of steel. In such cases a flux may be separately added or the raw alloying materials may be selected of such composition as to have in their gangue the necessary fluxing components.

Also a plurality of reducing agents may be used, such as a mixture of carbonaceous and metallic reducing agents or metal carbides, or several different metallic reducing agents. For instance, a ferro-silicon alloy containing carbon may be used, both its silicon and carbon contents being utilized for the reduction purpose. Also any reducing agents originally present in the steel bath may be effectively used, in which case during the reduction operation, a simultaneous refining of the original steel will take place. Also the fluxes added with the alloying-element-containing raw material will have the secondary effect of refining the steel of the metalloid contents, such as sulphur and phosphorus, simultaneously with the reducing operation.

If desired, after reduction of the alloying element or elements in the steel, a small quantity of additional ferro-silicon or ferromanganese may be added as a deoxidizing cleanser, before tapping, as in the common practice in making alloy steels. Also additions of other metals such as titanium, zirconium, copper, nickel, etc., may be used.

If desired these metals or scrap may be added between the successive chargings of the ore and reducing agent.

The advantages of this process of alloying are especially marked in the case of using silicon as a reducing agent, and producing steel or iron with a high alloy content and very low carbon content. As such an instance may be cited the manufacture of socalled "stainless" or "rustless" iron contain-

ing over 8% chromium and less than 0.1% carbon. Also the advantages of this process are apparent in the case of alloying a highly oxidizable and difficultly soluble element as uranium in steel. The alloying element being produced in the nascent state and directly in contact with the steel, the chances of its oxidizing or not dissolving are reduced to a minimum. Also, as the carbon content of the finished steel can be eliminated to any desired extent, simultaneously during the process of reducing, the exact percentage of carbon in the finished alloy steel can be arrived at more accurately by recarbonizing before tapping. In the case of metallic reducing agents being used their presence in the finished steel is practically eliminated by the action of fluxes and virtually completely removed by finally increasing the temperature. Thus by the process of this invention a steel of predetermined given composition can be more accurately produced than by the use of ferro-alloys. Also by this process, as the valuable alloying elements do not exist at any time in the metallic state, unless dissolved and alloyed in the steel itself, and as after their solution in the steel there is no occasion to subject such steel to an oxidizing process for removal of carbon, for instance, as in the older processes, there is no loss suffered through oxidation, rendering the process extremely economical. Also as the molten steel always carries an amount of reducing agent during the entire process, it is protected from absorbing oxides in it, thus producing a much cleaner finished steel in the solid state.

While the preferred method of carrying out my process has been specifically described, it is to be understood that the invention is not limited to all of the described details, but may be otherwise embodied in process of making alloy steels or irons, within the scope of the following claims:

I claim:

1. The process of making alloy steel or iron, comprising forming a molten bath of steel or iron having a metal layer and a slag layer, incorporating into the metal layer successive charges of a reducing agent the oxidation products of which render the slag more fluid and incorporating into the slag layer successive charges of an un-reduced compound of the alloying metal, and maintaining the bath at a temperature sufficient to cause a reaction between the reducing agent in the metal layer and the un-reduced compound of the alloying metal in the slag layer to thereby directly reduce the alloying metal in the bath, substantially as described.

2. The process of making chrome steel or iron, comprising forming a molten bath of steel or iron having a metal layer and a slag layer, charging into the bath successive charges of both a silicon reducing agent and

- chrome ore, the silicon reducing agent sinking through the slag layer and becoming incorporated in the metal layer and the chrome ore remaining in the slag layer and becoming incorporated therein, and maintaining the bath at a temperature sufficient to cause a reaction between the silicon in the metal layer and the chrome ore in the slag layer to thereby directly reduce chromium in the bath, substantially as described.
3. The process of making alloy steel or iron, comprising forming a bath of molten steel or iron having a metal layer and a slag layer, charging into said bath successive portions of both silicon and chrome ore and allowing sufficient time between successive charges to permit the silica produced by the oxidation of silicon to render the slag fluid, substantially as described.
4. The process of making alloy steel or iron, comprising forming a molten bath of steel or iron having a metal layer and a slag layer, adding to such bath in successive charges both an unreduced compound of the alloying metal and a reducing agent the oxidation products of which render the slag more fluid, and allowing sufficient time between successive charges for the reducing reaction to proceed to such point that the oxidation products of the reducing agent materially increase the fluidity of the slag, substantially as described.
5. The process of making alloy steel or iron, comprising forming a molten bath of steel or iron having a metal layer and a slag layer, and adding to such bath a reducing agent the oxidation products of which render the slag more fluid, an unreduced compound of the alloying metal and a fluxing material, each in successive charges alternating with charges of the other charged materials, substantially as described.
6. The process of making alloy steel or

iron, comprising forming a molten bath of steel or iron having a metal layer and a slag layer, adding to such bath a reducing agent the oxidation products of which render the slag more fluid, an unreduced compound of the alloying metal and a fluxing material, each in successive charges alternating with charges of the other charged materials, and periodically tapping off the dead slag, substantially as described.

7. The process of making alloy steel or iron, comprising forming a molten bath of steel or iron having a metal layer and a slag layer, adding to such bath in successive charges an unreduced compound of the alloying metal, a metalloid absorbing fluxing material and a reducing agent the oxidation products of which render the slag more fluid, and allowing sufficient time between charges for the reducing reaction to proceed to such point that the oxidation products of the reducing agent materially increase the fluidity of the slag, combined with a simultaneous refining of the iron and steel, substantially as described.

8. The process of making chrome steel or iron, comprising forming a molten bath of steel or iron having a metal layer and a slag layer, adding to such bath in successive charges chrome ore, a metalloid absorbing fluxing material and a silicon reducing agent, allowing sufficient time between successive charges for the reducing reaction to proceed to such point that the silica produced materially increases the fluidity of the slag, combined with a simultaneous refining of the iron or steel to take place, and periodically tapping off the dead slag, substantially as described.

In testimony whereof I have hereunto set my hand.

BYRAMJI D. SAKLATWALLA.